

# UNITED STATES PATENT OFFICE.

CHARLES A. HUTTINGER, OF LAKEWOOD, AND EDWARD RITTENHOUSE, OF CLEVELAND, OHIO, ASSIGNEES TO THE ACME WOOLEN-COTTON MILLS COMPANY, OF CLEVELAND, OHIO, A CORPORATION OF OHIO.

## PROCESS OF PRODUCING THREADS FROM VISCOSE.

1,367,603.

Specification of Letters Patent.

Patented Feb. 8, 1921.

No Drawing.

Application filed December 3, 1919. Serial No. 342,282.

To all whom it may concern:

Be it known that we, CHARLES A. HUTTINGER and EDWARD RITTENHOUSE, citizens of the United States, residents, respectively, of 5 Lakewood, county of Cuyahoga, and State of Ohio, and Cleveland, county of Cuyahoga, and State of Ohio, have invented new and useful Improvements in Processes of Producing Threads from Viscose, of which the following is a specification, the principle of 10 the invention being herein explained and the best mode in which we have contemplated applying that principle, so as to distinguish it from other inventions.

15 Our invention relates to processes of producing lustrous threads, etc., from viscose. This invention contemplates the production of a very soft and open thread. The invention relates particularly to the composition 20 of the bath in which the viscose is re-generated into cellulose hydrate.

The following description sets forth in detail certain steps illustrating the method of carrying out our invention such disclosed 25 steps constituting, however, but one of the various ways in which the principle of the invention may be utilized. In carrying out our improved process, we utilize a precipitating bath in the presence of a certain proportion 30 of molasses or incorporate the molasses with the bath. The proportion by weight of molasses may be from two to fifty per cent., but we have found that from ten to thirty per cent. gives very satisfactory results and 35 that substantially twenty per cent. by weight gives the best results.

Our precipitating bath, in addition to the molasses, consists of an aqueous solution of a salt and preferably of an aqueous solution 40 of sodium bisulfate because the latter is a by-product which can be bought comparatively cheaply. The relative proportions which we use are substantially ten (10) parts by weight water, six (6) parts bisulfate, and 45 four (4) parts molasses. Because of its impurities, and hence its cheapness, we preferably use molasses known as "third run." However, if a purer and more costly molasses were used, we do not contemplate the use of 50 a materially different proportion thereof

than that above set forth. The exact proportions of a very satisfactory bath will consist in one kilogram water, 631 grams sodium bisulfate and 410 grams molasses.

The thread obtained by spinning the multiple filaments of cellulose hydrate precipitated by a bath of this character disclosed is a product which has the necessary qualities as regards luster, strength and elasticity, and is also unusually soft and open. Our theory is that the extraordinary softness and openness is occasioned by the following physical action of the molasses while the filaments are setting in the precipitating bath. The molasses exteriorly coats the several strands of the viscose while the same is setting, possibly somewhat analogous to the coating of flour on a rolling board whereby the dough is prevented from sticking, so that the multiplicity of strands—from ten to 60 sixty or more, according to the thread produced,—do not stick or closely adhere when being twisted. This coating of molasses is washed off in the usual water washing after the skein is formed and the resultant product 65 is the very soft and open thread which has been mentioned.

What we claim is:

1. In the process of producing threads from viscose, the steps which consist, in introducing the latter in multiple streams into a precipitating bath composed of sodium bisulfate, water and molasses; and then spinning the resultant filaments, whereby a soft and open thread is obtained.

2. In the process of producing threads from viscose, the steps which consist, in introducing the latter in multiple streams into an aqueous solution of sodium bi-sulfate in the presence of molasses in proportion by weight of the bath of from ten (10) to thirty (30) per cent.; and then spinning the resultant filaments, whereby a soft and open thread is obtained.

3. In the process of producing threads from viscose, the steps which consist, in introducing the latter in multiple streams into a precipitating bath composed of substantially ten (10) parts by weight water; six (6) parts sodium bi-sulfate and four (4) 95

parts molasses; and then spinning the resultant filaments, whereby a soft and open thread is obtained.

4. In the process of producing threads from viscose, the steps which consist, in introducing the latter in multiple streams into a precipitating bath composed of substantially one thousand (1,000) parts by weight water; six hundred and thirty-one (631)

parts sodium bi-sulfate, and four hundred and ten (410) parts molasses; and then spinning the resultant filaments, whereby a soft and open thread is obtained.

Signed by us this 4th day of November, 1919.

CHARLES A. HUTTINGER.  
EDWARD RITTENHOUSE.